# EUROPEAN PATENT SPECIFICATION

(11) **EP 3 578 675 B1**
(45) Date of publication and mention of the grant of the patent: **13.07.2022**
(21) Application number: 19178372.9
(22) Date of filing: 05.06.2019
(51) Int. Cl.: C22C 18/00, C22F 1/16

(54) **HIGHLY MALLEABLE, DUCTILE ZINC STRIP**
HÖCHST VERFORMBARER, DUKTILER ZINKSTREIFEN
BANDE DE ZINC DUCTILE HAUTEMENT MALLÉABLE

(30) Priority: 07.06.2018 EP 18176438
(43) Date of publication of application: 11.12.2019
(73) Proprietor: Grillo-Werke Aktiengesellschaft, 47169 Duisburg (DE)
(72) Inventor: KROSS, Uwe, 47169 Duisburg (DE); KASPROWICZ, Bernd, 47169 Duisburg (DE); GOODEY, Trevor, Epping, Essex CM166FE (GB)
(74) Representative: dompatent von Kreisler Selting Werner - Partnerschaft von Patent- und Rechtsanwälten mbB

(56) References cited:
- CN-A- 102 453 926
- CN-A- 103 409 645
- PL-B1- 221 433
- US-A- 3 615 379
- KOKAWA H ET AL: "Observations of grain boundary fine structures in zinc by transmission electron microscopy", SCRIPTA METALLURGICA, ELSEVIER SCIENCE LTD., KIDLINGTON, GB, vol. 12, no. 4, 1 April 1978 (1978-04-01), pages 357-359, XP024134095, ISSN: 0036-9748, DOI: 10.1016/0036-9748(78)90299-5 [retrieved on 1978-04-01]

## Description

The present invention refers to a zinc strip comprising zinc as main component, wherein titanium and aluminium are alloyed together with the zinc. The obtained zinc strip is highly malleable and at the same time ductile. The zinc strip is free of lead. The zinc strip according to the present invention is ductile and the therefrom resulting high formability enables the skilled artisan to use the zinc strip especially in roofing applications.

Until today, usually lead is used in roofing applications, i.e. ceilings of dormers on a roof, transitions on a roof area etc. Lead is getting less and less accepted by the public due to its toxicity for humans. None of the alternative materials shows sufficient malleability and ductility for the above-mentioned applications.

Kokawa H. et al (Observations of grain boundary fine structures in zinc by transmission electron microscopy, Scripta Metallurgica, Elsevier, Bd 12, Nr. 4, 1.4.1978, S 357-359) discloses a rod made of zinc. The purity is 99.999%, which means that the sum of all impurities can amount to a maximum of 0.001%, i.e. 10 ppm. The content of Ti, Al, and Cu cannot be more than 10 ppm.

PL 221433 B1 discloses a Zn plate having a thickness of 10 mm. The Zn plate has an amount of at least 99.994% Zn and hence 60 ppm impurities. US 3,615,379 discloses a Zn alloy consisting of 99.9 to 99.995% Zn, 500 - 2500 ppm Ti, 50 to 500 ppm Al and 200 to 2000 ppm Cu.

Thus, it is the object of the present application to provide a zinc strip which is free of lead. At the same time, it shall be highly malleable and ductile. It should of course not be toxic. Surprisingly, it was found that alloying zinc with low amounts of titanium and aluminium enables the production of a highly malleable zinc strip.

Thus, in a first embodiment the present invention is solved by a zinc strip according to claim 1. In another embodiment, the present invention refers to the use of a respective zinc strip in the field of roofing. In another embodiment, the present invention refers to a method to produce a zinc strip with defined low amounts of titanium and aluminium.

Surprisingly it was found that a zinc strip with a defined low amount of titanium and aluminium, which are alloyed with the zinc, enables to produce a highly malleable, ductile zinc strip. Further surprisingly it was found that when producing a zinc strip, quite low temperatures of about 100° C are sufficient together with a high number of rolling passes to increase the malleability and ductility of the zinc strip.

The zinc strip of the present invention is obtained by alloying zinc with titanium and aluminium. The amount of titanium and aluminium should be quite low, namely it is 500 ppm or less and 100 ppm or less respectively. At the same time, the presence is needed to obtain the improved mechanical properties. The amount of titanium is at least 10 ppm and the amount of aluminium is at least 10 ppm as well.

In a preferred embodiment, the zinc strip further comprises copper. This copper will not be alloyed but is part of the used zinc. The amount of copper in the zinc strip is 500 ppm or less. Higher amounts of copper would result in worse mechanical properties, such as malleability and ductility.

Zinc usually comprises impurities. Known impurities are Pd, Cd, Fe and Sn.

The amount of impurities especially of the ones cited before is 0.05% by weight or less, especially 0.01% by weight or less, especially preferred 0.005% by weight or less, based on the total weight of the zinc strip. Surprisingly it was found that highly pure zinc with a defined low amount of copper can be alloyed with titanium and aluminium and the thus obtained alloy can be used to obtain zinc strips with good mechanical properties, especially malleability and ductility.

To have a low amount of total impurities, the zinc used to prepare the zinc strip is preferably high purity zinc according to classification Z1 of DIN EN 1179:2003. Using this highly pure zinc to produce the zinc strip enables to reduce and control the amount of total impurities and also to control the amount of copper in particular. Thus, in a preferred embodiment zinc of classification Z1 of DIN EN 1179:2003 is provided and titanium as well as aluminium are alloyed to obtain the zinc strip of the present invention which consists of zinc as main component. The amount of titanium is 500 ppm or less and the amount of aluminium is 100 ppm or less. Due to the use of the high purity zinc, also the amount of copper is 500 ppm or less.

In a preferred embodiment, the amount of titanium is 300 ppm or less, especially 100 ppm or less, preferably 50 ppm or less. The amount of aluminium is preferably 50 ppm or less. The amount of copper, where applicable, is preferably 300 ppm or less, preferably 100 ppm or less, especially 50 ppm or less, preferred 20 ppm or less.

The ratio of masses of aluminium and titanium being present in the zinc strip is preferably in the range of from 1:5 to 5:1, especially from 2:3 to 3:2, preferred from 1:2 to 2:1, it may also be 1:1, so that the amount of aluminium and titanium is approximately the same.

Amounts in ppm or percent by weight usually refer to the total weight of the zinc strip if not explicitly indicated different.

Using the high purity zinc and controlling the amount of titanium and aluminium and, where applicable, copper, enables as mentioned above to obtain a zinc strip with improved mechanical properties. Respective mechanical properties are for example tensile strength and yield strength. In the following Table 1, respective values are shown. Here, an inventive zinc strip is compared with known prior art substances.

**Table 1: Mechanical properties of different material**

| Material | tensile strength (Rm) | yield strength [Rp 0,2] |
|---|---|---|
| Titanium-Zinc^{∗} | min. 150 MPa | min. 100 MPa |
| Copper^{∗} | 220 - 260 MPa | max. 140 MPa |
| Stainless steel^{∗} | 500 - 700 MPa | ≥ 190 MPa |
| Galvanized steel^{∗} | 260 - 420 MPa | 120 - 220 MPa |
| Leadfree zinc strip according to the present invention | < 120 MPa | < 60 MPa |

| | | |
|---|---|---|
| ^{∗} not according to the invention | | |

Compared to known titanium zinc alloys, the zinc strip of the present invention differs especially in its chemical composition, where the amount of titanium, aluminium and copper, where applicable, are much lower than in known products. The chemical composition of titanium zinc compared with the zinc strip of the present application is shown in the following Table 2.

**Table 2: chemical composition (all values in % by weight)**

| | Titanium-Zinc (reference example) | Leadfree zinc strip according to the present invention |
|---|---|---|
| Copper | 0,08 - 1,0 % | < 0,002 % |
| Titanium | 0,06 - 0,2 % | < 0,005 % |
| Aluminium | max. 0,015 % | < 0,005 % |

In a preferred embodiment, the present invention refers to a zinc strip based on lead free zinc according to classification Z1 of DIN EN 1179:2003 which comprises 300 ppm or less titanium, 50 ppm or less aluminium as well as 300 ppm or less copper and the balance being zinc. In another preferred embodiment, the present invention refers to a zinc strip comprising zinc as main component, wherein the zinc is a high purity zinc according to Z1 of DIN EN 1179:2003, said zinc strip comprising 100 ppm or less titanium, 50 ppm or less aluminium as well as 100 ppm or less copper and the balance being zinc.

Also preferred is a zinc strip based on high purity zinc according to classification Z1 of DIN EN 1179:2003 comprising 100 ppm or less titanium, 50 ppm or less aluminium as well as 50 ppm or less copper and the balance being zinc. In another preferred embodiment, the zinc strip is based on high purity zinc according to classification Z1 of DIN EN 1179:2003 and further comprises 50 ppm or less titanium, 50 ppm or less aluminium as well as 20 ppm or less copper and the balance being zinc.

In another preferred embodiment, the zinc strip is based on a high purity zinc according to classification Z1 of DIN EN 1179:2003 further comprising titanium and aluminium, wherein the amount of titanium is 50 ppm or less, the amount of aluminium being 20 ppm or less and the amount of copper stemming from the zinc is 20 ppm or less and the balance being zinc. Further preferred is an embodiment in which a zinc strip being based on high purity zinc according to classification Zi of DIN EN 1179:2003 comprises 20 ppm or less titanium, 50 ppm or less aluminium as well as 20 ppm or less copper and the balance being zinc.

The zinc strip according to the present invention preferably has a thickness of 0.1 mm to 2.5 mm, especially 0.15 mm to 2.0 mm, preferably from 0.2 mm to 1.5 mm, preferred from 0.2 mm to 1.0 mm, especially preferred from 0.2 mm to 0.6 mm. These thicknesses enable good handability so that the zinc strip can be used in roofing applications, such as ceilings or transitions in roof areas, sealing a dormer of a roof, transitions in a roof area, roof ridges, eaves, chimney or wall connection, skylights, or to connect roof gutters.

It is within the invention, that the zinc strip may be coated with a colour so that it is not or at least hardly not visible after application. For a better application, it may also be possible that the zinc strip comprises an adhesive on one outer surface so that the strip can be applied to the area where it is used.

It is to be noted, that the thickness mentioned above refers to the thickness of the zinc strip only without a colour coating and/or an adhesive coating. The thickness of the colour coating, where present, is only several µm (usual values are in the range of 10 µm to 50 µm, especially 15 µm to 35 µm), so that it is not relevant for the thickness of the strip in total. The thickness of the adhesive, where present, is preferably within a range of from 0.1 mm to 1 mm, especially from 0.2 mm to 0.8 mm, preferred from 0.3 mm to 0.7 mm., especially preferred from 0.3 mm to 0.6 mm or to 0.5 mm. Preferably, the thickness of the adhesive is nearly the same or less than the one of the zinc strip. The ratio between the thickness of the adhesive and the thickness of the zinc strip is therefore in a preferred embodiment in a range of from 1:5 to 2:1, especially from 1:2 to 1:1.

The total thickness of a strip with adhesive is preferably in a range from 0.2 mm to 3.5 mm, especially from 0.3 mm to 2.5 mm, preferred from 0.5 mm to 1.5 mm, especially preferred from 0.6 mm to 1.2 mm, preferably from 0,7 mm to 1 mm. If the strip comprises not only an adhesive but also a colour coating the total thickness remains more or less the same.

The colour can be any suitable colour known by the skilled artisan. Suitable colours can be varnishes, such as alkyd varnish, epoxy resin varnish, polystyrene- or polyvinyl resin varnishes, phenolic varnish, urea varnish, melamine resin varnish or polyurethane varnishes. Varnishes based on polyurethane are especially preferred due to their high resistance against solvents, chemicals as well as whether influences. This enables a long colour during outdoor use.

In another preferred embodiment, the zinc strip comprises an adhesive on only one of the outer surfaces. The adhesive is added in such a way, that the zinc strip can be fixed on the area to be used. Thus, the adhesive may be coated on the complete out surface of the zinc strip. It is also within the invention, that the adhesive is on the other part of the one outer surface, such as in strips, points or that only specific areas to be connected with a specific basis are coated with an adhesive. It is to be noted, that the adhesive is only on one outer surface of the zinc strip, which is the surface to be added to the roof for example. The opposite surface will then be visible in use. This visible surface will of course not comprise any adhesive.

Suitable adhesives are for example adhesives based on acrylates, epoxides, phenolics, silicones, polyamides or adhesive tapes based on butyl. Acrylate adhesives and especially solvent free acrylate adhesives are especially preferred.

Preferred adhesives, especially the acrylate-based adhesives have the following advantages: High initial strength, good impact strength, high shear strength, UV resistance, good resistance against the influence of water, structural strength, goof wetting behaviour, can be applied to many surfaces, good resistance against changes in temperature, good resistance against influences of chemicals, as well as good aging resistance. Due to these advantages, adhesives based on acrylates are especially preferred, in particular those which are free of any solvents, as they enable a good adhesion in use and stability against all kind of weather effects.

In another embodiment, the present invention refers to a method of producing a zinc strip. The method includes providing zinc plates based on zinc. These plates further comprising titanium and aluminium where the amount of titanium is 500 ppm or less and the amount of aluminium is 100 ppm or less. To obtain such zinc plates, a zinc is alloyed together with titanium and aluminium in amounts such that the mentioned amounts are obtained. Preferably, the zinc is high purity zinc according to classification Z1 of DIN EN 1179:2003, preferably the amount of copper in the zinc is such that the amount of the zinc strip is 500 ppm or less.

The zinc plates are preferably made by continuous casting. In the beginning, the zinc plates are headed to a temperature of about 100° C or more. In the following, the plates are rolled as long as needed to obtain the thickness needed for using the strips in roofing applications.

The number of rolling passes needed to obtain the respective thickness is preferably 10 or more. It is advanteougous to have a discontinuous per pass reduction rate during the rolling process which is dependent on temperature and pressure during the rolling.

The final temperature of the rolling process is preferably about 50° C or more. The parameters of initial temperature, number of rolling passes, discontinuous prepass reduction rate as well as final temperature of the rolling process are relevant as all these features together and especially the initial temperature as well as the number of rolling passes enables the production of a zinc strip with high ductility and advantages mechanical properties. The method of the present invention enables the production of a zinc strip where the formation of coarse grains is avoided. This result in the excellent mechanical properties described above.

It is of course within the scope of the present invention that during the rolling process a rolling oil or an oil-based emulsion might be used.

Any embodiments disclosed in the specification can be combined with any other embodiment, even if not explicitly mentioned. Features disclosed for the method are also applicable for the zinc strip and vice versa.

## Claims

1. Zinc strip consisting of high purity zinc, wherein
the amount of titanium is at least 10 ppm and 500 ppm or less, and the amount of aluminium is at least 10 ppm and 100 ppm or less, and
wherein the balance is zinc, and usual impurities, especially Pb, Cd, Fe, and/or Sn, wherein the total amount of impurities amounts to 0.05 % by weight or less, based on the total weight of the zinc strip,
wherein the zinc strip optionally further comprises copper in an amount of 500 ppm or less, based on the total weight of the zinc strip.

2. Zinc strip according to claim 1, further comprising copper in an amount of 500 ppm or less, based on the total weight of the zinc strip.

3. Zinc strip according to claim 1 or 2, wherein the total amount of impurities amounts to 0.01 % by weight or less, preferably 0.005 % by weight or less, based on the total weight of the zinc strip.

4. Zinc strip according to any of claims 1 to 3, wherein the zinc is a high purity zinc according to classification Z1 of DIN EN 1179:2003.

5. Zinc strip according to any of claims 1 to 4, wherein the amount of titanium is 300 ppm or less, especially 100 ppm or less, preferably 50 ppm or less, based on the total weight of the zinc strip.

6. Zinc strip according to any of claims 1 to 5, wherein the amount of aluminium is 50 ppm or less, based on the total weight of the zinc strip.

7. Zinc strip according to any of claims 2 to 6, wherein the amount of copper is 300 ppm or less, preferably 100 ppm or less, especially 50 ppm or less, preferred 20 ppm or less, based on the total weight of the zinc strip.

8. Zinc strip according to any of claims 1 to 7, having a thickness of 0.1 mm to 2.5 mm, especially 0.15 mm to 2.0 mm, preferably from 0.2 mm to 1.5 mm, preferred from 0.2 mm to 1.0 mm.

9. Zinc strip according to any of claims 1 to 8, said strip being coated with a colour.

10. Zinc strip according to any of claims 1 to 9, said strip comprising an adhesive on one outer surface.

11. Use of a zinc strip according to any of claims 1 to 10 for sealing a dormer of a roof, transitions in a roof area, roof ridges, eaves, chimney or wall connection, skylights, or to connect roof gutters.

12. Method to produce a zinc strip according to any of claims 1 to 10 comprising:
a) providing zinc plates based on zinc and further comprising titanium, and aluminum, wherein the amount of titanium is 500 ppm or less, the amount of aluminum is 100 ppm or less,
b) warming the plates to a temperature of about 100 °C or more and
c) rolling the plates as long as needed to obtain the thickness needed for the using the strips in roofing applications.

13. Method according to claim 12, wherein the number of rolling passes in step c) amounts to 10 or more.

14. Method according to claim 12 or 13, wherein a discontinuous per pass reduction rate is obtained during the rolling process.

15. Method according to any of claims 12 to 14, wherein the final temperature of the rolling process is about 50 °C or more.

## Patentansprüche

1. Zinkstreifen, bestehend aus hochreinem Zink, wobei
die Menge an Titan wenigstens 10 ppm und 500 ppm oder weniger beträgt und die Menge an Aluminium wenigstens 10 ppm und 100 ppm oder weniger beträgt und
wobei der Rest aus Zink und üblichen Verunreinigungen, insbesondere Pb, Cd, Fe und/oder Sn, besteht, wobei die Gesamtmenge der Verunreinigungen 0,05 Gewichtsprozent oder weniger beträgt, bezogen auf das Gesamtgewicht des Zinkstreifens,
wobei der Zinkstreifen gegebenenfalls weiterhin Kupfer in einer Menge von 500 ppm oder weniger umfasst, bezogen auf das Gesamtgewicht des Zinkstreifens.

2. Zinkstreifen gemäß Anspruch 1, weiterhin umfassend Kupfer in einer Menge von 500 ppm oder weniger, bezogen auf das Gesamtgewicht des Zinkstreifens.

3. Zinkstreifen gemäß Anspruch 1 oder 2, wobei die Gesamtmenge der Verunreinigungen 0,01 Gewichtsprozent oder weniger, vorzugsweise 0,005 Gewichtsprozent oder weniger, beträgt, bezogen auf das Gesamtgewicht des Zinkstreifens.

4. Zinkstreifen gemäß einem der Ansprüche 1 bis 3, wobei das Zink ein hochreines Zink gemäß der Klassifikation Z1 von DIN EN 1179:2003 ist.

5. Zinkstreifen gemäß einem der Ansprüche 1 bis 4, wobei die Menge an Titan 300 ppm oder weniger, insbesondere 100 ppm oder weniger, vorzugsweise 50 ppm oder weniger, beträgt, bezogen auf das Gesamtgewicht des Zinkstreifens.

6. Zinkstreifen gemäß einem der Ansprüche 1 bis 5, wobei die Menge an Aluminium 50 ppm oder weniger beträgt, bezogen auf das Gesamtgewicht des Zinkstreifens.

7. Zinkstreifen gemäß einem der Ansprüche 2 bis 6, wobei die Menge an Kupfer 300 ppm oder weniger, vorzugsweise 100 ppm oder weniger, insbesondere 50 ppm oder weniger, vorzugsweise 20 ppm oder weniger, beträgt, bezogen auf das Gesamtgewicht des Zinkstreifens.

8. Zinkstreifen gemäß einem der Ansprüche 1 bis 7, der eine Dicke von 0,1 mm bis 2,5 mm, insbesondere 0,15 mm bis 2,0 mm, vorzugsweise 0,2 mm bis 1,5 mm, vorzugsweise 0,2 mm bis 1,0 mm, aufweist.

9. Zinkstreifen gemäß einem der Ansprüche 1 bis 8, wobei der Streifen mit einer Farbe überzogen ist.

10. Zinkstreifen gemäß einem der Ansprüche 1 bis 9, wobei der Streifen einen Kleber auf einer äußeren Fläche umfasst.

11. Verwendung eines Zinkstreifens gemäß einem der Ansprüche 1 bis 10 zur Versiegelung einer Gaube eines Dachs, von Übergängen im Dachbereich, Dachfirsten, Dachrinnen, Schornstein- oder Wandverbindung, Dachfenstern oder zum Verbinden von Dachrinnen.

12. Verfahren zur Herstellung eines Zinkstreifens gemäß einem der Ansprüche 1 bis 10, umfassend:
a) Bereitstellen von Zinkplatten, die auf Zink beruhen und weiterhin Titan und Aluminium umfassen, wobei die Menge an Titan 500 ppm oder weniger beträgt, die Menge an Aluminium 100 ppm oder weniger beträgt,
b) Erwärmen der Platten auf eine Temperatur von etwa 100°C oder mehr und
c) Auswalzen der Platten während einer Zeit, die benötigt wird, um die Dicke zu erhalten, welche benötigt wird, um die Streifen bei Dachanwendungen verwenden zu können.

13. Verfahren gemäß Anspruch 12, wobei die Anzahl der Walzdurchgänge in Schritt c) 10 oder mehr beträgt.

14. Verfahren gemäß Anspruch 12 oder 13, wobei während des Walzvorgangs eine diskontinuierliche Reduktionsrate pro Durchgang erhalten wird.

15. Verfahren gemäß einem der Ansprüche 12 bis 14, wobei die endgültige Temperatur des Walzvorgangs etwa 50°C oder mehr beträgt.

## Revendications

1. Bande de zinc constituée de zinc à haute pureté, dans laquelle
la quantité de titane est au moins 10 ppm et 500 ppm ou moins, et la quantité d'aluminium est au moins 10 ppm et 100 ppm ou moins, et
le reste étant du zinc et des impuretés usuelles, notamment du Pb, Cd, Fe, et/ou Sn, où la quantité totale des impuretés est de 0,05 % en poids ou moins, par rapport au poids total de la bande de zinc,
dans laquelle la bande de zinc éventuellement comprend en outre du cuivre en une quantité de 500 ppm ou moins, par rapport au poids total de la bande de zinc.

2. Bande de zinc selon la revendication 1, comprenant en outre du cuivre en une quantité de 500 ppm ou moins, par rapport au poids total de la bande de zinc.

3. Bande de zinc selon la revendication 1 ou 2, dans laquelle la quantité totale des impuretés est de 0,01 % en poids ou moins, de préférence 0,005 % en poids ou moins, par rapport au poids total de la bande de zinc.

4. Bande de zinc selon l'une quelconque des revendications 1 à 3, dans lequel le zinc est un zinc à haute pureté selon la classification Z1 de DIN EN 1179:2003.

5. Bande de zinc selon l'une quelconque des revendications 1 à 4, dans lequel la quantité de titane est 300 ppm ou moins, notamment 100 ppm ou moins, de préférence 50 ppm ou moins, par rapport au poids total de la bande de zinc.

6. Bande de zinc selon l'une quelconque des revendications 1 à 5, dans lequel la quantité d'aluminium est 50 ppm ou moins, par rapport au poids total de la bande de zinc.

7. Bande de zinc selon l'une quelconque des revendications 2 à 6, dans lequel la quantité de cuivre est 300 ppm ou moins, de préférence 100 ppm ou moins, notamment 50 ppm ou moins, de préférence 20 ppm ou moins, par rapport au poids total de la bande de zinc.

8. Bande de zinc selon l'une quelconque des revendications 1 à 7, ayant une épaisseur de 0,1 mm à 2,5 mm, notamment 0,15 mm à 2,0 mm, de préférence 0,2 mm à 1,5 mm, de préférence 0,2 mm à 1,0 mm.

9. Bande de zinc selon l'une quelconque des revendications 1 à 8, ladite bande étant recouverte d'une couleur.

10. Bande de zinc selon l'une quelconque des revendications 1 à 9, ladite bande comprenant un adhésif sur une surface extérieure.

11. Utilisation d'une bande de zinc selon l'une quelconque des revendications 1 à 10 pour sceller une lucarne d'un toit, des transitions dans une zone de toit, des faîtes de toit, des gouttières, une connexion de cheminée ou de mur, des vasistas, ou pour connecter des chéneaux.

12. Procédé pour produire une bande de zinc selon l'une quelconque des revendications 1 à 10, comprenant les étapes consistant à :
a) procurer des plaques de zinc basées sur zinc et comprenant en outre du titane, et de l'aluminium, la quantité de titane étant 500 ppm ou moins, la quantité d'aluminium étant 100 ppm ou moins,
b) chauffer les plaques à une température d'environ 100 °C ou plus, et
c) rouler les plaques pendant un temps nécessaire pour obtenir l'épaisseur appropriée pour l'utilisation des bandes dans des applications de toiture.

13. Procédé selon la revendication 12, dans lequel le nombre des passages de roulage dans l'étape c) est 10 ou plus.

14. Procédé selon la revendication 12 ou 13, dans lequel un taux de réduction par passage discontinu est obtenu pendant la procédure de roulage.

15. Procédé selon l'une quelconque des revendications 12 à 14, dans lequel la température finale de la procédure de roulage est environ 50 °C ou plus.
